

Patented Sept. 30, 1924.

1,509,872

## UNITED STATES PATENT OFFICE.

WALLACE J. MURRAY, OF BOSTON, MASSACHUSETTS, ASSIGNOR, BY MESNE ASSIGNMENTS, TO TODD PROTECTOGRAPH COMPANY, INC., OF ROCHESTER, NEW YORK, A CORPORATION OF NEW YORK.

## METHOD OF PRINTING SIZED PAPER.

No Drawing.

Application filed June 9, 1921. Serial No. 476,310.

*To all whom it may concern:*

Be it known that I, WALLACE J. MURRAY, a citizen of the United States, residing at Boston, in the county of Suffolk and State 5 of Massachusetts, have invented certain new and useful Improvements in Methods of Printing Sized Paper; and I do hereby declare the following to be a full, clear, and exact description of the invention, such as 10 will enable others skilled in the art to which it appertains to make and use the same.

The present invention relates to a method of printing permanent records in a manner 15 to prevent mechanical or chemical erasure and to a paper or fabric adapted to be so printed.

Repeated attempts have been made to devise a method of printing sized paper 20 which would preclude the possibility of a subsequent erasure of the printing either by mechanical or chemical means. Such a method has been more particularly sought in printing checks and similar instruments.

25 All previous methods, however, have been subject to certain inherent disadvantages which were sufficiently great to defeat the object sought for, namely the production of printed or written matter which could not 30 be removed by any known method. The disadvantages of previous methods may be briefly classified under two headings, the use of inks employing insoluble chemical-resistant coloring matter which is deposited 35 upon the surface of the paper or fabric in such a manner that it may be subsequently erased by mechanical methods and the use of soluble coloring matter which may penetrate somewhat into the body of the paper 40 or fabric but is capable of being removed by other chemicals.

I have discovered that it is possible to 45 initially impregnate sized paper such as is used for checks and to thereafter employ an ink which will react with the material in the paper to form insoluble coloring matter distributed throughout the body of the paper according to any desired form of predetermined design. The coloring matter 50 so formed cannot be removed by mechanical erasure without destroying the body of the paper and by a suitable selection of materials a fast color may be formed which cannot be removed by chemical means. In

addition I have discovered that the ink used 55 in printing or writing upon the paper can be caused to penetrate throughout the body of a sized paper by the employment of an oil base as a vehicle. The use of this oil base permits the printing to be accomplished 60 with metal type, plates, or with a pen, as desired, in either case the ink penetrating the body of the paper to substantially its entire depth without spreading sufficiently 65 to impair the legibility of the printing or writing. Ordinary printing inks have an oil vehicle in which is suspended insoluble pigments. In printing the pigment is deposited on the surface, while the vehicle may penetrate the paper to a varying degree. My 70 new process takes advantage of this property of oil to penetrate a sized paper, and in my new inks the materials are dissolved rather than suspended in the vehicle. In this way I can carry into the body of the 75 paper reagents which react with materials initially contained in the paper, precipitating insoluble colored pigments throughout the body of the paper.

As one illustration of my new method 80 of printing sized paper, an azo color can be produced within the body of the paper by first treating the paper with a nitrite such as sodium nitrite, or other bodies capable of yielding free nitrous acid, and then 85 printing the prepared paper with an ink consisting of a solution of a primary amine and a developer, such as a phenol, in a fatty acid or other vehicle capable of penetrating a sized paper and containing in addition a 90 free acid. As an example a glyceride containing a free fatty acid or other acid may be employed. The acid in the ink vehicle liberates nitrous acid from the nitrite or 95 other substance capable of yielding nitrous acid in the paper, which in turn diazotizes the primary amine dissolved in the ink vehicle, this diazotized amine reacting or coupling with the developer to precipitate the insoluble azo color in the body of the paper. The azo color may be made faster 100 by mordanting, that is, treatment with metallic salts or other means familiar to the art of textile dyeing. Such further agents may be included in the paper, in the 105 ink, or may be used in an after-treatment.

It is possible by this method to produce a large number of colors. For example, if

- the paper is initially treated with sodium nitrite and is then printed with an ink consisting of beta-naphthol and dianisidine dissolved in oleic acid, dianisidine blue is produced in the body of the paper by the resulting reactions. Owing to the red color of the oleic acid the combination of the dianisidine blue therewith may produce a purple or brown in the paper.
- 10 It should be understood by those skilled in the art that the oil solvent is intended to embrace fatty acids, glycerides, hydro-carbon and other vehicles capable of penetrating a sized paper, and in addition of liberating an acid from the nitrite with which the paper is impregnated. With the exception of fatty acids the vehicle is in itself incapable of liberating nitrous acid from nitrates and in all other cases an acid must be included among the reagents dissolved in the oil vehicle.
- 15 20

I claim:

1. A method of making permanent records on sized paper which consists in impregnating the paper with a reagent capable of yielding nitrous acid and applying to the surface of the paper an ink capable of penetrating the sized paper and reacting with the reagent to liberate nitrous acid and precipitate a pigment within the body of the paper.
- 25 30
2. A method for making permanent records on sized paper, which consists in initially impregnating the paper with a re-

agent capable of yielding nitrous acid, and applying to the surface of the paper an ink consisting of a solution of an amine and a developer in an oil capable of penetrating the paper, and liberating nitrous acid from the reagent contained in the paper.

40

3. A method for making permanent records on sized paper, which consists in impregnating the paper with a nitrite, and applying to the surface of the paper an ink consisting of a solution of a primary amine and a developer in a fatty acid.

45

4. A method for making permanent records on sized paper, which consists in impregnating the paper with a nitrite, and subsequently applying to the surface of the paper an ink consisting of a solution of a primary amine and a phenol in a fatty acid.

50

5. A method of printing sized paper, which consists in initially impregnating the paper with a nitrite, drying the paper, and thereafter applying to the surface of the paper an ink consisting of a solution of a primary amine and a phenol in oleic acid.

55

6. A method of printing sized paper, which consists in impregnating the paper with sodium nitrite, drying the paper, applying to the surface of the paper an ink consisting of a solution of dianisidine and beta-naphthol in oleic acid.

60

7. A sized paper impregnated with a nitrite.

WALLACE J. MURRAY.